

## UNITED STATES PATENT OFFICE.

JUDSON A. DE CEW, OF MOUNT VERNON, NEW YORK.

## LUBRICATING EMULSION.

No Drawing. Application filed April 18, 1919, Serial No. 291,030. Renewed January 26, 1922. Serial No. 532,037.

*To all whom it may concern:*

Be it known that I, JUDSON A. DE CEW, a subject of the King of Great Britain, and native of the Dominion of Canada, residing at Mount Vernon, New York, have invented a new and useful Improvement in Lubricating Emulsions, of which the following is a specification.

The following invention relates to improvements in the lubricating value of emulsions used in machine shops on cutting tools. Although aqueous emulsions are used to cool and lubricate cutting tools with fairly satisfactory results, I have discovered that owing to the very high pressure at the point of the tool and the high temperatures reached at the cutting edge, the lubricating value of the oil particles is not as great as it might be, because the viscosity of the oil is so greatly reduced by these high temperatures when it actually comes between the metal and the edge of the tool, that it is only able to partially reduce the friction existing at this surface.

The object of this invention is to attach to the oily particles in the emulsion, certain solid lubricants which will be carried with the emulsion to the point of contact between the cutting tool and the work and this will supply the means for keeping the surfaces lubricated irrespective of the high temperatures and pressures existing at the edge of the tool.

To accomplish this result, I use in the emulsifying process, a small quantity of very fine graphite or other solid or colloidal lubricant. The solid lubricant is mixed with the oil and then emulsified by any of the methods that have been described herefore, the object being to produce a special kind of emulsion in which there are two liquid and one solid phases and in which the distribution is uniform. I am aware that colloidal graphite has been used, blended

with oil to improve its lubricating properties and also that suspensions of graphite in water have been used for lubrication but I believe that it is a new invention to produce uniform emulsions in which both oil and graphite are dispersed in an aqueous medium.

I do not limit myself to the use of graphite as other solid lubricants such as talc may be employed. A specific example is as follows: Three ounces of graphite and six ounces of talc are completely mixed in two gallons of oil. This mixture is then put in a measuring tank and emulsified into one hundred gallons of water.

What I claim as my invention is:

1. A lubricating dilute emulsion of a water insoluble solid and water insoluble liquid particles dispersed in an aqueous medium the solid particles, being enclosed by the liquid particles.

2. A dilute emulsion having therein a water insoluble oil, graphite and water, the graphite particles being enclosed by the oil particles.

3. A dilute emulsion having therein a water insoluble oil, a water insoluble solid lubricant and water, the solid particles being enclosed by the liquid particles.

4. A new lubricating product comprising particles of a water insoluble oil highly dispersed in an aqueous medium and enclosing minute particles of water insoluble solid lubricant.

5. A process of making emulsions containing an unemulsified water insoluble solid lubricant, which consists in emulsifying a water insoluble oily material in which the solid lubricant is enclosed, into an aqueous medium.

In testimony whereof, I, the said JUDSON A. DE CEW, have signed my name to this specification this 16th day of April 1919.

JUDSON A. DE CEW.